

## UNITED STATES PATENT OFFICE

2,237,682

## GREASE CONTAINING ASPHALT

Lester W. McLennan, Richmond, Calif., assignor  
to Union Oil Company of California, Los Angeles, Calif., a corporation of California

No Drawing. Application August 24, 1935, Serial  
No. 37,755. Renewed January 16, 1939

5 Claims. (Cl. 252—39)

This invention relates to greases of the cup grease type, particularly to cup greases in which asphaltic materials are included.

For certain uses, such as in saw mills and the like, it has been found that ordinary cup greases, such as calcium soap grease, are not entirely satisfactory, whereas if a refined asphalt is included an additional stickiness and body is imparted to the grease, and where an oxidized or airblown asphalt is added in suitable proportions, it produces a firmer grease of much better body which has a more plastic structure, as well as an unusually black luster, both of which features render the grease highly preferable. For example, about 15% of an airblown asphalt added to a calcium soap grease results in a grease of such suitable texture and consistency.

The invention may therefore be said to reside in a cup grease, that is, a calcium soap grease, containing a quantity of oxidized asphalt, and particularly an airblown asphalt in quantity sufficient to provide a firmer more plastic structure than that imparted by steam blown or ordinary residual asphalts. The invention applies also to other greases or oils thickened with soaps and containing oxidized asphalts for the purposes stated.

Asphaltic cup greases and the like of the stated character possess their improved consistency apparently by reason of improved adhesive characteristics.

In preparation of an asphaltic cup grease according to the present invention, the calcium soap grease is made up according to approved conventional practices, the soap stocks being preferably a mixture of about 85% prime tallow and 15% oleic acid, although other soap stocks may be used as obvious to the skilled grease maker. Saponification is effected in an open kettle with hydrated lime, together with a small quantity of mineral oil if desirable to improve working consistencies. Following saponification, the required amount of mineral oil for the desired grease is introduced and worked into the soap, and water is added to attain the necessary hydration as required in calcium soap greases, whereupon airblown asphalt is added with agitation until the asphalt has been completely assimilated by the hot grease. The amount of asphalt so introduced is preferably such as to constitute about 15% of the product. The temperature is then adjusted and the grease is drawn into containers.

A desirable airblown asphalt is an asphalt which has been produced by airblowing, as dis-

tinguished from steam blowing, and also as distinguished from ordinary residual asphalts. A typical airblown asphalt has a melting point of 145–155° F. by the standard ball and ring method A. S. T. M. D-36-26, a penetration of 30–40 at 77° F. by the standard A. S. T. M. method D-5-25. Harder or softer specimens however, may be used. The mineral oil used may be any appropriate oil for grease-making purposes such as one having a Saybolt Universal viscosity at 100° F. of 200 seconds. The amount of oil in the final product will depend of course upon the consistency of the grease desired. Thus, in a typical sample of light grease there may be about 72% oil and 12% calcium soap and reaction products together with about 1% water, whereas for a medium grease the oil content may be about 68% and for a heavy grease about 58%, the soap and water contents being correspondingly increased.

10 A finished light cup grease according to this invention possesses the following typical composition:

|                                                            | Per cent<br>by weight |
|------------------------------------------------------------|-----------------------|
| 25 Calcium soap                                            | 11.2                  |
| Glycerin                                                   | 1.0                   |
| Mineral lubricating oil (Say. Vis. 200 sec.<br>at 100° F.) | 71.69                 |
| 30 Free fat                                                | 0.3                   |
| Free alkali                                                | 0.01                  |
| Airblown asphalt as above described                        | 15.0                  |
| Water                                                      | 0.8                   |

Heavier greases are made merely by decreasing the proportion of oil with a corresponding increase in the proportion of soap and water to about 58% oil and 2% water for a heavy grease.

35 A satisfactory operating procedure comprises charging to a kettle about 740 lbs. of a soap stock consisting of about 85% prime tallow and 15% oleic acid, together with a little over 100 lbs. of hydrated lime, about 25 lbs. of water, and if desired, a small proportion of the mineral oil, for example about 200 lbs. This batch is heated with agitation until saponification is complete. This may be a matter of two or three hours. The temperature will be run up to about 230° F. The presence of the oil enables the soap to be kept in a soft condition without the formation of lumps. Having obtained proper saponification, part of the oil is added rapidly and worked into the soap until the temperature is reduced to about 200° F. and the soap content is reduced to perhaps 25% or 30%. Thereupon the small quantity of water required in a calcium grease is added for proper

hydration of the grease and in the case of lighter greases the rest of the lubricating oil is then worked in. The above described airblown asphalt is then added to the grease in small lumps and the grease is paddled until the asphalt has been completely taken up. The temperature of the grease is then adjusted to a proper drawing temperature, as determined by factors well known in the art of cup grease manufacture, and drawn off into containers.

In addition to producing calcium soap greases containing airblown asphalt above described, other metal soaps may be employed to produce corresponding cup greases, such variations being made in water content and certain steps of procedure as would be well understood by the skilled grease maker.

Grease as produced according to this invention has imparted thereto by the asphalt an unusually black luster that cannot be obtained with other asphalts, and at the same time a firmer, more plastic, and generally more desirable grease structure is obtained than with other asphalts. Also such oxidized asphalts produce greases more suitable for various heavy uses than non-asphaltic or other asphaltic greases. Not only may the ordinary solid greases be produced, but the so-called liquid greases may also be produced by increasing the quantities of lubricating oil, and for some uses the quantity of lubricating oil may be further increased to yield an oil only slightly thickened by relatively small amounts of soap and asphalt. Except as the quantity of lubricating oil varies the consistency, the characteristics imparted by the asphalt are substantially the same throughout the mentioned range of lubricants.

The addition of asphalt as above described is particularly effective in the case of greases which are resistant to water, such as calcium soap greases. As to the quantity of oxidized asphalt to be employed in the various greases, the invention is by no means limited to the 15% given in the example, although this has been found to be a very desirable proportion. Greases may be prepared which contain more or less asphalt, for example as high as 20% or 25%, and as low as 10% or even 2%. Probably in general, for commercial uses, practical limits would be between

about 10% and 20%. Of course in the cases of liquid or semi-liquid greases and in the more fluid oils above mentioned, the asphalt percentages would necessarily run correspondingly lower.

It is therefore to be understood that the disclosures here made are to be considered as illustrative and not as limiting except as required by the state of the prior art.

10 I claim:

15 1. A grease comprising a major proportion of mineral oil thickened with a calcium soap in amount sufficient to impart cup grease consistency, and between about 10% and 25% of an airblown asphalt having a melting point according to the A. S. T. M. ball and ring method between about 140° F. and about 155° F. and a penetration at 77° F. of 30 to 40 according to the A. S. T. M. method.

20 2. A cup grease comprising a major proportion of mineral oil thickened to cup grease consistency with a water-insoluble soap imparting water resistant characteristics to the grease, and between about 10% and 25% of airblown asphalt having a melting point according to the A. S. T. M. ball and ring method between about 140° F. and about 155° F. and a penetration at 77° F. of 30 to 40 according to the A. S. T. M. method.

25 3. A grease comprising in excess of about 58% of mineral oil thickened with at least about 11% of calcium soap and containing approximately 15% of airblown asphalt having a melting point according to the A. S. T. M. ball and ring method between about 140° F. and 155° F. and a penetration at 77° F. of 30 to 40 according to the A. S. T. M. method.

30 4. A grease comprising a major proportion of mineral oil thickened to cup grease consistency with a water-insoluble soap imparting water resistant characteristics to the grease, and between about 10% and 25% of a normally solid airblown asphalt.

35 45 5. A grease comprising a major proportion of mineral oil thickened with a calcium soap in amount sufficient to impart cup grease consistency, and between about 10% and 25% of an airblown asphalt solid under normal conditions.

LESTER W. McLENNAN.